



# UNITED STATES PATENT OFFICE.

CLAUD E. FULLER, OF KANSAS CITY, MISSOURI.

## METHOD OF TREATING POROUS BLOCKS.

1,231,007.

Specification of Letters Patent. Patented June 26, 1917.

Application filed July 13, 1916, Serial No. 109,027. Renewed May 14, 1917. Serial No. 168,595.

*To all whom it may concern:*

Be it known that I, CLAUD E. FULLER, a citizen of the United States, residing at Kansas City, in the county of Jackson and 5 State of Missouri, have invented a certain new and useful Improvement in Methods of Treating Porous Blocks, of which the following is a specification.

My invention relates to improvements in 10 methods of treating porous blocks.

It relates particularly to the treatment of blocks by impregnation of the same with a suitable filling material, such as asphalt.

In the ordinary treatment of blocks, such 15 as bricks, the purpose has been to fill the pores as completely as possible with the filling material.

The object of this invention is to provide a method of treatment which will require 20 less asphalt than will the ordinary treatment and which at the same time will contain a maximum amount of filling material in the outer portion of the block, while the central portion will contain no filling material, or at least the pores will not be filled 25 in such central portion. This treatment affords economy of manufacture, while producing a block that will have maximum wearing qualities.

30 In the preferred embodiment of my invention, the blocks, the pores of which contain air or other suitable compressible fluid, are first heated so as to expand the blocks, following which the blocks are subjected to 35 pressure greater than atmospheric, thereby compressing the fluid contained within the pores, after which the blocks are immersed in their heated condition, and while still under pressure, in the liquid filling material, which is a liquid that will solidify at 40 ordinary atmospheric pressure and temperatures, such as asphalt or other suitable bituminous material. The immersed blocks are then subjected to still greater pressure

45 than that first applied, thereby compressing the fluid in the pores and forcing the compressible fluid, such as air, to the central portion of the block. The remaining pores of the block will be filled with filling material, such as asphalt. The pressure is then 50 reduced and the blocks are suddenly cooled in any desired manner, such as by immersion in cold water; by spraying with cold water, by being subjected to a draft of cold

air, or by any other cooling means which 55 will suddenly cool the blocks.

Upon being suddenly cooled, the blocks will first contract on their outer portions, the contraction extending from outside inwardly. In like manner the solidification 60 of the asphalt will be from the outside inwardly, thereby permitting the compressed air or other compressible fluid, which is in the central portions of the blocks, to force the asphalt, which is contained in the pores 65 of the intermediate portions of the blocks, and which is still liquid, to fill such voids as occur due to the contraction of the solidifying outer asphalt, the latter having greater contraction and expansion than the blocks, 70 if the blocks are bricks.

A portion of the inner liquid asphalt will thus be forced outwardly thereby making denser the outer portions of the blocks where density is required for the purpose of better 75 withstanding wear. Thus the completed block will have its outer portion filled with a maximum of asphalt, the central portion will only contain air, as asphalt is not needed in this portion, and the intermediate portion will not be filled to saturation. The cost of production of the blocks will thus be 80 less than with blocks which are fully saturated with asphalt, while the wearing qualities of the blocks will be increased owing to 85 the more complete saturation of the outer portions thereof.

In the accompanying drawings I have 90 illustrated an apparatus with which my invention may be carried into effect.

Figure 1 is an end elevation, partly broken away of my improved apparatus.

Fig. 2 is an enlarged vertical sectional view of the check valve, controlling the bypass, and parts connected therewith.

Fig. 3 is a horizontal sectional view of a block which has been impregnated but not cooled.

Fig. 4 is a horizontal sectional view of a block which has been impregnated and the 100 cooling operation finished.

Similar reference characters designate similar parts in the different views.

1 designates the treating chamber in which the blocks or bricks 2 are immersed in the 105 liquid filling material, such as asphalt, which is liquefied by heat in a melting tank 3, which is preferably located above the treat-

ing chamber 1, and which with the latter is located within a suitable inclosure 4, shown in dotted lines, and which serves as a heating chamber.

5 Any suitable means may be employed to heat the chamber 1 and tank 3 to a temperature above the melting point of the filling material. In the chamber 1, I have shown in the lower part thereof steam heating coils 10 5, which may be employed for heating the interior of the chamber.

One end of the chamber 1 is provided with a removable end or door 6 which may be removed so as to permit a car 7 carrying the 15 blocks or bricks 2 to run into and out of the chamber 1 on a track comprising rails 8 which are supported respectively on longitudinal supports 9 supported on the inner wall and bottom portion of the chamber 1.

20 10 designates a conductor, the upper end of which is connected with the bottom of the tank 3 and the lower end of which is connected to a reversible pump 11, of any suitable type and which, preferably is located, 25 as is the pipe 10, in the inclosure 4 so as to prevent chilling of the filling material as it passes therethrough. A conductor 12 has one end connected with the other port of the pump 11; the other end of said conductor 30 being connected with the upper side of a sediment tank 13, the upper side of which is connected by a vertical pipe 14. The sediment tank 13 is located within the inclosure 4 and below the chamber 1, and is provided 35 at one end with a removable closure 15, which upon being removed, permits the removal of sediment from the tank 13.

The pump 11 is provided with a driving shaft 16, which is also the driving shaft of a 40 duplex reversible engine 17 of any suitable type, and which is supplied by steam through a pipe 18 which is connected with an automatic governor 19, such as the well known Gardner governor, which in turn is connected by a conductor 20 with the conductor 12, and which automatically controls the passage of steam through the pipe 18 to the engine 17, the governor 19 in turn being controlled by the pressure in the treating chamber 1 which is communicated to the governor 19 by means of the pipe 14, sediment tank 13, and conductors 12 and 20. When the pressure in the chamber 1 falls below a predetermined point, the governor 19 will permit more steam to be supplied to the engine 17 through the steam pipe 18, thereby increasing the speed of operation of the pump 11 and the pressure in the chamber 1 as well as the amount of asphalt supplied to the 55 latter.

In the conductor 10 is a shut-off valve 21 having a controlling stem 22 which extends to the exterior of the inclosure 4.

The conductor 10 is provided with a 60 branch 23 which leads through the inclosure

wall 4 to the atmosphere and which is provided with a shut-off valve 24.

A priming conductor 25 is connected at its upper end to the bottom of the tank 3, and at its lower end is connected to the conductor 10 at a point intermediate of the pump 11 and branch 23. In the conductor 25 is a shut-off valve 26 which is provided with a controlling stem 27 which extends through the inclosure wall 4.

75 When the pump 11 is used to pump air into the chamber 1, the valve 21 is closed and the valves 24 and 26 are opened, the latter valve being opened so as to permit a small quantity of asphalt to pass from the tank 3 through the conductor 25 into the lower portion of the conductor 10 and thence into the pump 11 for the purpose of priming and sealing the latter.

In order that the pressure may not rise 85 above a pre-determined point in the chamber 1, there is provided a by-pass 28, opposite ends of which respectively connect with the conductors 12 and 20. Within the by-pass 28 is located a check valve 29, Fig. 90 2, which opens outwardly, with respect to the chamber 1, and which is provided with a horizontal stem 30 which extends through a stuffing box 31 and through the inclosure wall 4. The outer end of the stem 30 is 95 screw-threaded and is slidably mounted in a bracket 32 secured to the outer side of the inclosure wall 4. A coil spring 33 encircles the stem 30 and has its outer end bearing against the bracket 32 and its inner end bearing against a nut 34 which is adjustably mounted on the threaded part of the stem 30. By adjusting the nut 34, the tension of the spring 33 may be varied so as to increase or decrease the pressure applied 105 to the valve 29 for holding said valve seated.

When the pressure in the chamber 1 arrives at the pre-determined point, the valve 29 will be opened against the pressure of the spring 33, thus permitting asphalt to 110 flow from the conductor 12 past the pump 11 into the conductor 10 through the by-pass 28.

In the operation of my invention, the car 7 containing the blocks or bricks 2 is 115 run into the chamber 1, after which the latter is closed. Preferably before being run into the treating chamber 1, the blocks or bricks 2 are pre-heated to approximately 350 degrees, when asphalt is to be used as a filling material, following which the blocks or bricks are quickly transferred to the treating chamber 1.

The tank 3 and chamber 1 having been heated to a temperature above the melting point of the asphalt contained in the tank 3, and the valves 21 and 26 being closed, the valve 24 is opened and the engine 17 started, thus operating the pump 11 in a manner such that air will be drawn through 125 130

the branch 23 and conductor 10 into the pump 11 and by the pump forced through the conductor 12, sediment tank 13, and pipe 14 into the treating chamber 1. The 5 valve stem 27 may be turned so as to open the valve 26 to permit sufficient asphalt to pass from the tank 3 through the conductor 25 and the conductor 10 into the pump 11 for the purpose of sealing and priming the 10 latter.

15 The pump 11 is operated until a sufficient air pressure greater than atmospheric is provided in the chamber 1 and in the pores of the blocks or bricks 2.

15 The valve 24 is then closed and the valve 20 stem 22 turned so as to open the valve 21, the pump 11 still being driven by the engine 17 in the same direction in which it has been running. Asphalt will now be pumped

20 from the tank 3 through the conductor 10, pump 11, conductor 12, sediment tank 13 and pipe 14 into the treating chamber 1. This pumping operation is continued until the blocks or bricks 2 are fully immersed

25 and until the desired increased pressure required for forcing the liquid asphalt into the pores of the outer portions of the blocks has been obtained. At this time each block 2 will have a central portion 35, the pores

30 of which will contain only compressed air, or such other compressible fluid as may have been forced into the pores of the blocks in the first pumping operation. The pores of the remaining portion of the block will be 35 impregnated with liquid asphalt in that part indicated by 36 in Fig. 3.

The engine 17 is then reversed, thereby reversing direction of operation of the pump 11, upon which the asphalt will be 40 pumped back into the tank 3 through the pipe 14, tank 13, conductor 12, pump 11, and conductor 10. The valves 21 and 26 are then closed and the door of the chamber 1 opened so that the car 7 may be run 45 out of the chamber 1 and suddenly cooled by immersion in water.

The outer portion of each block will first be cooled, thereby solidifying the asphalt and the solidification and cooling will progress from the outer side inwardly. As the asphalt solidifies in the outer portion of the block, it will contract to a greater extent than the blocks or bricks 2, thereby leaving voids which will be filled by the 55 liquid asphalt still contained and not yet solidified in the intermediate portion between the central portion 35 and the outside of the block or brick, the compressed fluid in the portion 35 forcing the inner liquid 60 asphalt outwardly, thereby filling the voids occasioned by the solidification and contraction of the asphalt in the pores of the outer portion of the block.

When the cooling operation has been completed, so that all of the asphalt in the

block has been solidified, the outer portion of the block designated by 37 in Fig. 4, will be more densely filled with asphalt than the inner portion 36. The outer portion of the block, which is subjected to wear 70 and the action of the elements will be densely filled with asphalt, the central portion 35 will contain no asphalt, and the intermediate portion 36, Fig. 4, will have its pores only partly filled with the asphalt. 75

By means of the process just described, blocks will be produced which will have a maximum amount of asphalt in their outer portions, thereby imparting maximum durability to the blocks while at the same time 80 effecting a minimum cost of treatment due to the relatively small amount of asphalt employed as a result of the compressed air contained within the central portion of each block.

85 In the treatment of blocks or bricks which are exceptionally porous so as to already contain sufficient air for effecting the function, the preliminary air pumping step may be eliminated.

90 Instead of immersing the blocks after impregnation with the asphalt, the blocks may be suddenly cooled by being subjected to a blast of cold air, which may be blown upon them through a conductor 38, Fig. 1, connected with a suitable source of supply, not shown, and containing a shut off valve 39 which is closed excepting during the air cooling operation. The conductor 38 has one end connected to the upper side of the 100 chamber 1.

95 Or the blocks may be suddenly cooled by spraying with a cold liquid, such as water discharged through a conductor 40, Fig. 1, one end of which is connected to the upper 105 side of the chamber 1 and the other end of which is connected with a source of supply, not shown. The conductor 40 contains a shut off valve 41 which is closed excepting during the spraying operation. 110

I do not limit my invention to the structure shown nor to the precise steps described, as modifications, within the scope of the appended claims may be made without departing from the spirit of my invention. 115

What I claim is:—

1. The method consisting in forcing at pressure greater than atmospheric into the pores of a porous block a substance liquefied by heat and which solidifies at ordinary temperatures, and then suddenly cooling the block while it is under pressure substantially atmospheric. 120

2. The method consisting in forcing at pressure greater than atmospheric into the pores of a porous block a substance liquefied by heat and which solidifies at ordinary temperatures, and then reducing the pressure and suddenly cooling the block. 125

3. The method consisting in forcing at 130

pressure greater than atmospheric into the pores of a porous block liquid bitumen which solidifies at ordinary temperatures, then reducing the pressure, and suddenly cooling the block.

4. The method consisting in forcing at pressure greater than atmospheric into the pores of a porous block liquid bitumen which solidifies at ordinary temperatures, then reducing the pressure to substantially atmospheric, and then suddenly cooling the block.

5. The method consisting in forcing liquid asphalt into the pores of a porous block at a pressure greater than atmospheric, then reducing the pressure, and then suddenly cooling the block.

6. The method consisting in forcing liquid asphalt into the pores of a porous block at a pressure greater than atmospheric, then reducing the pressure to substantially atmospheric, and then suddenly cooling the block.

25 7. The method consisting in heating a porous block, then forcing at a pressure greater than atmospheric into the pores of the block a substance liquefied by heat and which solidifies at ordinary temperatures, then reducing the pressure, and then suddenly cooling the block.

30 8. The method consisting in heating a porous block, then forcing at a pressure greater than atmospheric into the pores of the block a substance liquefied by heat and which solidifies at ordinary temperatures,  
35 then reducing the pressure to substantially atmospheric, and then suddenly cooling the block.

9. The method consisting in heating a porous block, then forcing at a pressure greater than atmospheric liquid bitumen which solidifies at ordinary temperatures, then reducing the pressure and then suddenly cooling the block.

10. The method consisting in heating a  
porous block, then forcing at a pressure  
greater than atmospheric into the pores of  
the block liquid asphalt, then reducing the  
pressure, and then suddenly cooling the  
block.

50 11. The method consisting in heating a porous block, then forcing at a pressure greater than atmospheric into the pores of the block liquid bitumen which solidifies at ordinary temperatures, then reducing the pressure to substantially atmospheric, and then suddenly cooling the block.

12. The method consisting in heating a porous block, then forcing at a pressure greater than atmospheric into the pores of the block liquid asphalt, then reducing the pressure to substantially atmospheric, and then suddenly cooling the block.

13. The method consisting in compressing the air in the pores of a porous block, then forcing into the pores at a still greater pres-

sure a substance liquefied by heat and which solidifies at ordinary temperatures, then reducing the pressure, and then suddenly cooling the block.

14. The method consisting in compressing the air in the pores of a porous block, then forcing into the pores at a still greater pressure a substance liquefied by heat and which solidifies at ordinary temperatures, then reducing the pressure to substantially atmospheric, and then suddenly cooling the block. 70 75

15. The method consisting in compressing the air in the pores of a porous block, then forcing into the pores at a still greater 80 pressure liquid bitumen which solidifies at ordinary temperatures, then reducing the pressure, and then suddenly cooling the block.

16. The method consisting in compressing 85  
the air in the pores of a porous block, then  
forcing into the pores at a still greater pres-  
sure liquid bitumen which solidifies at ordi-  
nary temperatures, then reducing the pres-  
sure to substantially atmospheric, and then 90  
suddenly cooling the block.

17. The method consisting in compressing the air in the pores of a porous block, then forcing into the pores at a still greater pressure liquid asphalt, then reducing the pressure, and then suddenly cooling the block. 95

18. The method consisting in compressing the air in the pores of a porous block, then forcing into the pores at a still greater pressure liquid asphalt, then reducing the pressure to substantially atmospheric, and then suddenly cooling the blocks.

19. The method consisting in heating a porous block, then compressing the air in the pores of the block, then forcing into the pores at a still greater pressure a substance liquefied by heat and which solidifies at ordinary temperatures, then reducing the pressure, and then suddenly cooling the block. 105.

20. The method consisting in heating a 110 porous block, then compressing the air in the pores of the block, then forcing into the pores at a still greater pressure a substance liquefied by heat and which solidifies at ordinary temperatures, then reducing the 115 pressure to substantially atmospheric, and then suddenly cooling the block.

21. The method consisting in heating a porous block, then compressing the air in the pores of the block, then forcing into 120 the pores at a still greater pressure liquid bitumen which solidifies at ordinary temperatures, then reducing the pressure, and then suddenly cooling the block.

22. The method consisting in heating a 125 porous block, then compressing the air in the pores of the block, then forcing into the pores at a still greater pressure liquid bitumen which solidifies at ordinary temperatures, then reducing the pressure to substan- 130

tially atmospheric, and then suddenly cooling the block.

23. The method consisting in heating a porous block, then compressing the air in the pores of the block, then forcing into the pores at a still greater pressure liquid asphalt, then reducing the pressure, and then suddenly cooling the block.

24. The method consisting in heating a porous block, then compressing the air in the pores of the block, then forcing into the pores at a still greater pressure liquid asphalt, then reducing the pressure to substantially atmospheric, and then suddenly cooling the block.

25. The method consisting in compressing fluid in the pores of a porous block, then forcing into the pores at a still greater pressure a substance liquefied by heat and which solidifies at ordinary temperatures, then reducing the pressure, and then suddenly cooling the block.

26. The method consisting in forcing at a pressure greater than atmospheric into the pores of a porous block, the pores of which contain a compressible fluid, a liquid substance which solidifies at ordinary temperatures, then reducing the pressure, and suddenly cooling the block.

27. The method consisting in forcing at a pressure greater than atmospheric into the pores of a porous block, the pores of which contain a compressible fluid, liquid bitumen which solidifies at ordinary temperatures, then reducing the pressure, and suddenly cooling the block.

28. The method consisting in forcing at a pressure greater than atmospheric into the pores of a porous block, the pores of which contain a compressible fluid, liquid asphalt, then reducing the pressure and suddenly cooling the block.

29. The method consisting in compressing

a compressible fluid in the pores of a porous block, then forcing into the pores at a still greater pressure a liquid which solidifies at ordinary temperatures, then reducing the pressure and then suddenly cooling the block.

30. The method consisting in compressing a compressible fluid in the pores of a porous block, then forcing into the pores at a still greater pressure liquid bitumen which solidifies at ordinary temperatures, then reducing the pressure, and then suddenly cooling the block.

31. The method consisting in compressing a compressible fluid in the pores of a porous block, then forcing into the pores at a still greater pressure liquid asphalt, then reducing the pressure, and then suddenly cooling the block.

32. The method consisting in heating a porous block, then compressing in the pores of the block a compressible fluid, then forcing into the pores at a still greater pressure a liquid which solidifies at ordinary temperatures, then reducing the pressure, and then suddenly cooling the block.

33. The method consisting in heating a porous block, then compressing in the pores of the block a compressible fluid, then forcing into the pores at a still greater pressure liquid bitumen which solidifies at ordinary temperatures, then reducing the pressure, and then suddenly cooling the block.

34. The method consisting in heating a porous block, then compressing in the pores of the block a compressible fluid, then forcing into the pores at a still greater pressure liquid asphalt, then reducing the pressure, and then suddenly cooling the block.

In testimony whereof I have signed my name to this specification.

CLAUD E. FULLER.